

# UNITED STATES PATENT OFFICE.

LEE H. BOWMAN, OF MUNHALL, PENNSYLVANIA, ASSIGNOR TO CARNEGIE STEEL COMPANY, OF PITTSBURG, PENNSYLVANIA, A CORPORATION OF NEW JERSEY.

## METHOD OF MAKING ARMOR-PLATE.

996,558.

Specification of Letters Patent. Patented June 27, 1911.

No Drawing. Application filed May 18, 1908, Serial No. 433,499. Renewed November 22, 1910. Serial No. 593,724.

To all whom it may concern:

Be it known that I, LEE H. BOWMAN, of Munhall, Allegheny county, Pennsylvania, have invented a new and useful Method of 5 Making Armor-Plate, of which the following is a full, clear, and exact description.

My invention relates to the manufacture of face hardened armor plate and is designed to provide an improved method by 10 which the back portion of the plate is given a greater tensile strength than that present in the plates as now made.

The invention consists primarily in subjecting the back portion of the plate to a 15 heat treatment which will give a crystalline structure in this back, preferably extending to about the middle of the plate; then applying the heat treatment to the face of the plate for hardening. In the heat treatment 20 for the face hardening of the plate, I have found that this crystalline back portion will be converted into fiber which gives a structure of higher tensile strength than that now afforded to present plates.

25 In carrying out my invention, I preferably follow standard practice in casting and forging, after which the plate may be carburized and reforged or not as desired, and then fiber the plate in the ordinary manner 30 by heat treatments, such as are well known. The plate may then be shaped and machined if desired. At this point I then introduce my new step, which step preferably consists in bedding the face portion of the plate in 35 loam, introducing the plate into a furnace, and heating the back of the plate up to a temperature of about 950° C. This heat should be carried to above the point of 40 recalescence and may be varied above such temperature according to the chill desired.

The plate should be given a longer heat treatment than that now used for face-hardening or the temperature should be increased. In this step, the back and preferably about half of the body of the plate, is 45 brought to a high temperature, or above the point at which steel hardens, after which the plate is taken out of the furnace and quenched, preferably in water. The back of 50 the plate is then given the crystalline structure which may extend to any desired depth, preferably to about half the thickness of the plate. The plate is then face-hardened in any desirable manner, as for example by

bedding the back in loam, placing the plate 55 in the furnace and heating its face to about 950° C. During this heat treatment of the face, the back of the plate will be brought up to a temperature of about 450° to 600° C., when the plate is then taken out and 60 quenched, preferably in water. The crystalline back portion of the plate will be converted into a strong fibrous structure, while at the same time the face will be given the desired hardness. In this operation, both 65 faces are preferably quenched by water sprays, although they may not be applied for the same duration on each face. If the temperature of the back of the plate is slightly higher than desired when the plate 70 is taken out of the furnace, the spray may be applied to the face of the plate, and when the back has been brought down to the proper temperature the spray is then applied to it.

75 The advantages of my invention result from the steps of forming a crystalline structure on the back portion of the plate and then converting this structure into a strong, fibrous structure. It is found in 80 practice that this increases the ballistic resistance of the plate. The crystalline structure of the back portion of the plate may be converted into fiber either during the face hardening or before it.

85 While my process is applied advantageously to face-carburized armor plate, it may be applied to homogeneous plates, in which case the homogeneous back would be converted into a strong fiber back by heat 90 treatment.

I claim:

1. In the manufacture of armor plate, the steps consisting in taking a fibered steel plate, heating the back portion of the plate 95 to convert it into a crystalline structure while retaining the face portion in annealed or fibered condition, quenching the same, and then converting said crystalline structure into a strong, fibrous structure by heat 100 treatment and quenching; substantially as described.

2. In the manufacture of armor plate, the steps consisting in forming a fibered steel plate, heating the back portion of the plate 105 up to above the recalescence point while retaining the face portion in annealed or fibered condition, quenching the plate, then

heating the face portion to above the recalescence point while the back portion of the plate is heated to a temperature not exceeding that at which annealing takes place and then quenching the plate to convert the crystalline structure of the back into a strong fibrous structure; substantially as described.

3. The method of making face hardened armor plate, consisting in heating the back portion of a fibered or annealed plate to the proper temperature while retaining the face portion in annealed or fibered condition,

and then quenching to produce a crystalline structure in said back, and then converting 15 the crystalline structure of the back into a strong fibered portion by heating the face portion of the plate to the proper hardening temperature and quenching the plate; substantially as described.

In testimony whereof, I have hereunto set my hand.

LEE H. BOWMAN.

Witnesses:

G. M. VIERS,  
H. M. CORWIN.